

Aug. 18, 1931.

C. B. COATES ET AL.

1,819,148

ELECTRICAL APPARATUS

Filed March 21, 1928



INVENTORS  
Charles B. Coates  
Clarence J. Dresser  
BY

S. A. D. Nickerson  
ATTORNEY.

## UNITED STATES PATENT OFFICE

CHARLES B. COATES AND CLARENCE J. DRESSER, OF CLEVELAND, OHIO, ASSIGNEES  
TO CHICAGO PNEUMATIC TOOL COMPANY, OF NEW YORK, N. Y., A CORPORATION  
OF NEW JERSEY

## ELECTRICAL APPARATUS

Application filed March 21, 1928. Serial No. 263,564.

This invention relates to electrical apparatus, particularly electrical motors of the alternating current induction type without commutators or brushes. More specifically 5 it relates to an improved form of rotor for such motors, especially small motors for electrical tools of the portable or hand type such as are used for drilling, tapping, reaming, riveting, screw driving, nut running, stud 10 setting, etc.

Among the objects of the invention are to improve the performance, to increase the reliability and to avoid certain weaknesses in motors for portable electrical tools, to develop 15 a rotor for such tools characterized by high sustained speed, high torque, indestructibility and reduced weight, to determine upon suitable alloys for cast windings and end rings for securing the above results and 20 to fix upon the relative proportions and dimensions of the winding and end rings. Other objects will be apparent from the detailed description which follows.

While it has heretofore been proposed to 25 construct rotors having the conducting leads or bars and the end rings in one piece, no attempt has been made to adapt the same for use with portable hand operated tools where power and sustained high speed together with light weight are important factors under the exacting requirements of present day mass production methods. U. S. Patent No. 1,647,633, issued November 1, 1927, to C. E. Johnson, proposes to use an aluminum alloy for cast windings and end rings 30 but for motors above 5 H. P. and with features intended to reduce the amount of current required for starting. The prior art however including the Johnson patent fails 35 to give details regarding what metal or metallic alloy should be used for the casting operation and what the bar and end ring areas must be if the cast rotors are to equal or to exceed the performance of motors having 40 rotors of standard construction, i. e., with bar or wire windings. By extended experimentation and research work the more desirable alloys for the specific purpose were determined upon and during the development 45 period it was discovered that a formula could

be devised for determining the end ring areas which would give substantially maximum results with the chosen alloys.

When the experimental work was begun, it was found that better results could be obtained with an aluminum alloy than with pure aluminum. Trials with an aluminum alloy containing copper were encouraging. Good results were secured with aluminum alloys containing from 4% to 16% of copper 60 with best results at 8% to 10% of copper. On account of the difference in conductivity, the cast conductor bars of the rotor had to be made approximately two times the size of the copper conductor bars or coils ordinarily used 65 in a motor of given capacity. Hence the shape of the slots in the rotor core became important and extended tests established that slots expanding toward the periphery of the core with substantially radial sides gave the 70 necessary bar area without excessive impairment of the magnetic densities of the teeth of the rotor core. Open slots were found to be preferable in that this arrangement minimized the zigzag leakage between the teeth 75 of the rotor core. The area of conductors having been established, a formula was eventually worked out for determining the cross sectional area of the end rings, this formula containing a constant K with a 80 preferential value of .4 but with a permissive variation of from .36 to .46 without serious impairment of the operating characteristics of the motor.

In order to illustrate the invention a concrete embodiment thereof is shown in the accompanying drawings in which:

Fig. 1 is a longitudinal sectional view through the improved rotor with a removable shaft shown in broken outline, the section 90 being taken substantially on the broken line 1-1 of Fig. 2.

Fig. 2 is a transverse sectional view substantially on the line 2-2 of Fig. 1, the shaft being omitted.

As indicated the rotor core is made up of a plurality of iron plates 3 providing a laminated structure, which plates have a series of slots 4 disposed symmetrically adjacent their peripheries. Each slot has a restricted open- 100

ing through the periphery thus leaving teeth 5 of substantial size on the plates alternating with the slots therein. The plates are assembled in face engagement with the slots 4 thereof in substantial register in accordance with the usual practice. While maintained in this position, conductor bars 6 and end rings 7 integral with the rods 5 are cast in one piece and in one operation upon the armature core 3.

If the casting is to be done in sand molds an alloy of aluminum with from 4% to 16% of copper is used, the preferred alloy containing aluminum 92% to 90% and copper 8% to 10%, the molten alloy being arranged to enter at the bottom of the mold and to pass upwardly through the aligned slots 4 in the laminated core body 3 expelling the air and other gasses ahead of the molten metal. If the rotor is to be die cast the copper content of the alloy may be reduced and silicon added. A preferred alloy giving substantially the results of the preferred aluminum-copper alloy with the same bar and end ring areas consists of aluminum 94½%, copper 2½%, silicon 3%.

As shown in Fig. 2, the slots in the core plates are of substantial size, being formed to contain substantially two times as much of the cast alloy as of copper either in bar or wire form. To secure an opening for such an increased mass of the conducting material without reducing permissible magnetic densities of the teeth 5 between the slots 4, each slot is relatively small and rounded toward the axis of the armature and expands or enlarges outwardly with straight sides which are substantially radii of the armature plates, the slot being constricted adjacent the periphery of the plate to a narrow slot opening. The slot then becomes substantially shovel or spade shape. The entire slot including the restricted peripheral opening is filled with the cast alloy as indicated, the alloy and the peripheral surface of the core plates 3 forming a continuous annular surface.

To reduce slip to a minimum, so that high operating speeds and maximum horse-power can be obtained and sustained, end rings of certain cross sectional area were required and it was found to be possible to determine such area very exactly for motors of differing sizes and capacities by the formula

$$A = \frac{anK}{N}$$

in which  $A$  indicates the cross sectional area of the end ring,  $a$  the cross sectional area of one of the rotor slots,  $n$  the number of such slots, and  $N$  the number of stator poles of the motor.  $K$  is a constant with .4 as a preferred value although this value may vary from .36 to .46 with but slight effect upon the operating characteristics of the motor.

A preferred shape of the cast end rings 7

is illustrated in Fig. 1, wherein the rings are shown as tapered annuli having their bases upon the end rotor plates and wholly covering the slots 4 save for the restricted peripheral openings thereof between the teeth 5 of the plates.

Rotors constructed in accordance with the present invention and utilizing the aluminum alloys herein specified, are much lighter than copper bar or wire wound rotors. They are substantially indestructible and the integral union of the cast bars and end rings makes any loosening of the rotor plates, such as occurs with copper bar rotors, wholly impossible. Likewise and for the same reason the unfortunate effects of a loosened coil in a wire wound rotor are avoided. An additional advantage results from the smooth contour of the improved rotor, particularly when provided with tapered end rings as shown which prevent dirt and grit from lodging on the rotor and cutting through the stator windings as happens with motors used in grinding and other abrading or polishing operations. Most important is the fact that rotors formed in accordance with the present invention and utilizing the alloys and the proportioned dimensions herein disclosed are found to develop greater horse-power, higher torque, and a higher sustained speed than corresponding copper bar and wire wound rotors.

While the invention has been herein disclosed in what is now considered a preferred form, it is to be understood that the invention is not limited to the exact details thereof but covers all changes, modifications and adaptations within the scope of the appended claims.

We claim as our invention:

1. A rotor for induction motors having a slotted core and having conductor bars and end rings cast in one piece upon said core of an alloy comprising approximately nine parts aluminum and one part copper, said bars being of uniform shape and of substantial size in cross section, namely rounded toward the axis of the rotor with diverging straight sides conforming substantially to radii of the rotor and covered at the outer wide portion save for a central narrow part which extends to and forms a part of the peripheral surface of the rotor, each said ring being in the form of an annulus having its sides extending axially and tapered toward each other, the base of each ring engaging an end face of the core and covering the body portion of said bars, the cross sectional area of each ring equalling the cross sectional area of all the bars divided by the number of poles of the motor and multiplied by .4.

2. A rotor for induction motors designed for high sustained speed and high torque, said rotor having a slotted core and having

conductor bars and end rings cast in one piece upon said core, said bars being of substantial size in cross section and coverd as to their outer portions by said core save for a narrow part which extends to and forms a part of the peripheral surface of the rotor, said rings being in the form of annuli spaced from the periphery of the rotor and from the rotor shaft with wide bases engaging the ends of said core and covering the body portions of said bars, said rings extending outwardly from said core with smooth converging tapered sides and terminating in rounded ends thereby to cause dust and grit to be thrown off so as to prevent the cutting through of stator winding.

Signed by us at Cleveland, in the county of Cuyahoga and State of Ohio, this 17th day of March, 1928.

CHARLES B. COATES.  
CLARENCE J. DRESSER.

25

30

35

40

45

50

55

60

65